

May 3, 1966

R. S. MacCAFFRAY, JR., ETAL

3,248,825

METHOD OF REMOVING GLOSS FROM MAGNESIUM MOLD SURFACE

Filed Jan. 13, 1964



INVENTORS  
Rex S. MacCaffray, Jr.  
Kenneth E. Hawkins  
BY  
D. S. DeLoach and Son  
ATTORNEYS

**1**

3,248,825

**METHOD OF REMOVING GLOSS FROM  
MAGNESIUM MOLD SURFACE**

Rex S. MacCaffray, Jr., Boiling Springs, and Kenneth E. Hankins, Carlisle, Pa., assignors to C. H. Masland & Sons, Carlisle, Pa., a corporation of Pennsylvania  
Filed Jan. 13, 1964, Ser. No. 337,433  
7 Claims. (Cl. 51—281)

The present invention relates to a method of treating the molding surface of a magnesium or magnesium alloy mold to reduce the lustre and produce a uniform surface.

The purpose of the invention is to brush the molding surface of a magnesium alloy mold with an alkaline abrasive compound in a slurry in a suitable liquid such as water at or below ambient temperature to remove any surface film which may have resulted from etching of the surface and produce a surface having less lustre and more uniformity.

A further purpose is to protect a magnesium or magnesium alloy mold surface while it is exposed to water and while it is being abraded, by an alkaline solution, suitably containing zinc oxide in dispersion.

A further purpose is to stabilize the molding surface of a magnesium or magnesium alloy mold.

A further purpose is to produce a controllable degree of delustering of the mold surface.

A further purpose is to improve the surface appearance of products molded in a magnesium or magnesium alloy mold by removing a coating which tends to form on the surface and which produces a variable high gloss on the molded object in different areas.

A further purpose is to rub the scrubbing brush over a cake of suitable alkaline soap, for example Fels Naphtha or P & G laundry soap, before applying it to the slurry in the mold, thus increasing the alkalinity, aiding in dispersing the zinc oxide or other abrasive, acting as a detergent to remove oil and grease from the surface and tending to protect against any corrosive action which might be exerted by chlorine or the like in city water.

A further purpose is to incorporate in the slurry from 0.2% to 15% on the weight of the solids of a hard abrasive such as aluminum carbide or silicon carbide in a size range below 100 microns and preferably in a size range of 50 to 100 microns and thus accelerate the speed of abrading.

Further purposes appear in the specification and in the claims.

The drawing is a diagrammatic transverse section of a magnesium or magnesium alloy mold which is useful in explaining the invention.

For many purposes it is desirable to mold plastic against a base material, which may be wood, metal, paper fiber, textile material, or of some other character, whether in the partially prepared or finished form. For example, plastic moldings may be applied on furniture, on doors, windows, chair rails, or other building components, on paper for reinforcing or ornamental purposes, on fiberboard for ornamental or reinforcing purposes, and on textile fabrics, particularly carpets and rugs, for reinforcing on places of exceptional wear, as for example stair treads and risers, entrances to rooms, and in front of furniture and the like where frequent wear is encountered. In the making of automobile carpet it is common practice to apply protection to the surface of the carpet at locations where the heel of the driver's foot will be placed and other locations where executive wear might be encountered.

It has previously been discovered that formulations of plastic, rubber or synthetic rubber can to advantage be molded on the surface of a base material such as carpet, wood fiber, paper, metal or the like.

**2**

The material used is generally referred to as a plastic and may be of any of the well-known types, such as phenol-formaldehyde, urea-formaldehyde and others of the thermosetting plastics, or it may be one of the thermoplastics including polyvinyl chloride, polyvinyl acetate, polyvinyl chloride acetate and also it may be one of the elastomeric materials similar to rubber or synthetic rubber including buna S, buna N and others. Olefinic plastics of the type of polyethylene and polypropylene may also be used.

For many purposes the most widely used plastics for these applications are polyvinyl chloride plastisols, of the character well known in the art which are gelled and fused under heat preliminary to cooling, at which time they adhere to the fabric to form a solid plastic.

As shown in the drawing, very desirable molds are obtained from magnesium or magnesium base alloys. The alloys are 90 or more percent magnesium, usually 95 percent or more magnesium, the balance being small alloying additions of such metals as aluminum, zinc and manganese. Typical magnesium alloys of which the molds are desirably made are PE alloy which contains 3.25 aluminum and 1.2 percent zinc, the balance being magnesium, all percentages being by weight. Another suitable magnesium base alloy for making such molds is AZ31B which has a nominal composition by weight of 3 percent aluminum, 1 percent zinc and 0.2 percent manganese, balance magnesium.

These alloys are commonly machined by chemical machining, etching with a suitable acid, desirably dilute nitric acid, usually according to techniques described in one or more of the following patents:

Easley and Swayze, U.S. Patents 2,940,763 to 2,940,767; Hopkins and Easley, U.S. Patent 2,828,194; Fishaver, U.S. Patent 2,940,836; Easley and Hopkins, U.S. Patent 2,979,387; and Easley and Fishaver, U.S. Patent 3,023,138.

It will be evident also that the mold can be mechanically machined in whole or in part.

One of the undesirable effects of the process of manufacture previously employed is that the mold has an uneven glossy or shiny surface which produces a variable undesirable glossy surface on the plastic molding.

One of the problems presented is that further etching techniques which might remove this surface may present the difficulty of loss in refinement of detail of the contour or corrosion of the magnesium or magnesium alloy. Furthermore, if the usual etching techniques are used for this purpose, while they remove the objectionable layer, they create an objectionable glossy surface themselves.

We have discovered that it is possible to remove the variable glossy layer while protecting the molding surface of the magnesium or magnesium alloy against corrosion and at the same time to produce a very desirable uniform less lustrous surface.

In the preferred embodiment of the invention we pour on the active surface of the mold a slurry of finely divided alkaline abrasive in a suitable liquid, preferable water.

The abrasive is preferably zinc oxide, but other suitable alkaline abrasives which may be used are magnesium oxide, magnesium carbonate or calcium carbonate. The alkaline abrasive should be finely divided, that is, it should have a mesh of a size of 0.5 to 5 microns and preferably 0.5 to 1 micron, and the particles should be free from sharp corners.

In addition to the alkaline abrasive it is desirable to use a soap, suitably a commercial laundry soap having excess of alkali (Fels Naphtha or P & G soap is a suitable example). This performs the functions of removing oil and grease, dispersing the abrasive, and further

maintaining the alkalinity and protecting against any harmful effect from chlorine or other components in domestic water supplies. The quantity of soap should be sufficient to give a little lather. Other detergents should not be used as they may attack the magnesium. In some cases it is desirable also to add a hard abrasive of the character of aluminum carbide or silicon carbide, which should be present in the range of from 0.2% to 5% of the total solids in the slurry, the percentage being measured by weight. The particle size is the finest suitable for optical grinding, which is desirably of a size of 50 to 100 microns. The hard abrasive speeds up de-lustering.

It is advisable to use water and abrasive at or below ambient temperature, so as to reduce undesirable activity by way of attacking the magnesium.

Instead of water, other suitable liquids can be used, such as ethyl alcohol, methyl alcohol, Stoddard solvent and any other liquid which will not injure the magnesium surface under the conditions.

The action of the liquid is intended to be physical rather than chemical as it functions as a carrying medium.

The abrasive is mixed in the liquid in great excess to form a slurry which will suitably be of milky or creamy consistency.

The preferred technique is to place the active mold surface horizontal and uppermost, pour the slurry of alkaline abrasive and liquid on the mold surface, and then to rub it manually with a brush. The preferred brush is a nylon bristle scrubbing brush of the character well known in the art and commonly used for scrubbing fixtures and floors in the kitchen and bathroom. Brushes of tampico fiber were used with success, but they deteriorated rapidly. Pig bristle brushes may also be used. The bristle size is suitably of the order of 20 to 50 denier.

We find that the brush strokes should preferably be in the advancing circular direction and the downward force on the brush should be of the order of 5 to 15 pounds per scrubbing brush.

#### Example I

A magnesium alloy mold **20** of PE alloy of the shape shown in the drawing has an active mold face **21** produced by chemical machining or etching, surrounded by a rim **22**. Active mold face **21** has numerous contours or projections **23** which are intended to form recesses in the molded object.

As produced it has an objectionable nonuniform gloss on the active surface which is believed to be due to a coating which forms as a result of the chemical etching or other machining.

We pour into the mold and on the active face a slurry **24** of milky consistency of ordinary city tap water and zinc oxide shaken up at ambient temperature. The particle size of the zinc oxide was 0.5 to 1 micron, rounded corners. The slurry is rubbed with a nylon bristle scrubbing brush using an advancing rotary motion and a downward force of about 10 lbs. The time taken in scrubbing each portion of the surface is about five seconds and the total time therefore depends on the size of the mold.

The result obtained is that the active face of the mold is of reduced and more uniform gloss without any appreciable change in dimension and without any loss in definition of the contours **23**. The surface instead becomes uniform which produces a similar uniform finish on the molded heel pad or other object.

#### Example II

An attempt was made to add various anionic detergents in the procedure of Example I and it was found that they were unusable because they immediately marked the surface. Trisodium phosphate and various polyphosphates proved to be bad.

#### Example III

In applying the technique of Example I the wet brush was rubbed over an alkaline laundry soap, of the character of Fels Naphtha soap or P & G laundry soap, when first applying it to the mold. This promoted the wetting of the magnesium surface and reduced the time of processing appreciably.

#### Example IV

The technique of Example I was carried out except that from 0.2% to 15% of a hard grit on the weight of the solids was incorporated in the slurry. The hard grit used was optical aluminum carbide abrasive having a particle size of the order of 50 to 100 microns and in one example it formed 5% of the solids. This reduced the time of the operation to the extent of about  $\frac{1}{2}$  and further reduced the gloss.

#### Example V

The technique of Example I was carried out using the soap according to Example III and using the hard abrasive according to Example IV. This further slightly cut the time of the operation.

#### Example VI

The procedure of Example I is carried out using sodium bicarbonate instead of zinc oxide. The action in making the luster uniform is less rapid than in the case of Example I.

#### Example VII

The procedure of Example I is carried out using sodium carbonate instead of zinc oxide. The action is similar to that in Example I except that it proceeds less rapidly.

In view of our invention and disclosure variations and modifications to meet individual whim or particular need will doubtless become evident to others skilled in the art, to obtain all or part of the benefits of our invention without copying the method shown, and we therefore claim all such insofar as they fall within the reasonable spirit and scope of our claims.

Having thus described our invention what we claim as new and desire to secure by Letters Patent is:

1. A method of reducing and making more uniform the lustre on a mold surface of a mold of the class consisting of magnesium and magnesium alloys, which comprises scrubbing the mold surface with a brush in the presence of a slurry of an alkaline abrasive in a liquid to modify the surface and produce a uniform finish of lower lustre.

2. A method of claim 1, in which the alkaline abrasive is a material of the class consisting of zinc oxide, magnesium oxide, magnesium carbonate and calcium carbonate and the liquid is water.

3. A method of claim 2, which comprises further introducing an alkaline soap into the slurry.

4. A method of claim 3, which comprises further incorporating into the slurry from 0.2% to 15% of a hard abrasive of a particle size not in excess of 100 microns.

5. A method of claim 1, which comprises incorporating into the slurry an alkaline soap.

6. A method of claim 1, which comprises incorporating into the slurry from 0.2% to 15% of a hard abrasive having a particle size finer than 100 microns.

7. A method of claim 1, which comprises scrubbing with an alkaline abrasive of the class consisting of zinc oxide, magnesium oxide, magnesium carbonate and calcium carbonate in water at a temperature not in excess of ambient temperature.

#### References Cited by the Examiner

UNITED STATES PATENTS

2,853,409 9/1958 Helling ----- 51-322 X

75 LESTER M. SWINGLE, Primary Examiner.